

## UNITED STATES PATENT OFFICE.

ALBERT ELSENHANS, OF ESSEN, GERMANY.

## ROTARY MACHINE SIEVE OF WIRE GAUZE PARTICULARLY FOR PAPER MACHINES.

No Drawing. Application filed May 18, 1926, Serial No. 110,009, and in Germany October 28, 1924.

In the endless sieves or wire cloths of paper making machines the rapid wear and tear to which they are subjected, is principally caused by the friction produced by the various rollers over and around which they are passed under working conditions and also that produced by the suction boxes and cleaning appliances. The wire cloths are also continually bent and straightened again in their passage round the rollers and are furthermore subjected continuously to tensile strains in the direction of their length. In consequence of these actions particularly the incessant bending and straightening, the material of the wire cloth becomes gradually destroyed, and it is the warps in particular of the wire gauze which suffer under these circumstances, whereas the destructive action on the wires of the weft is less.

The wires hitherto commonly used for the wire cloths of paper making machines are mostly composed of bronze or a material similar to bronze, and these wire cloths consequently possess only a very limited length of life. The use of steel wires, although they are considerably stronger than the aforesaid wires and better able to resist the above mentioned mechanical influences, is not convenient as this material rusts, whereby not alone is its destruction accelerated, but the material treated easily becomes contaminated. Recently highly alloyed improved steels have been produced, which do not rust and in addition to great hardness possess an extraordinary degree of toughness, whereby they are afforded a power of resistance to breakage and wear which is not possessed by any other material. It has also been already proposed to make wire cloths for papermaking machines of improved steel, as its pre-eminent properties make it much more suitable for the purpose than any other kind of wire. Its use is however not by any means economical, because its market price is so high (approximately ten times that of bronze when in the form of wire gauze) that the advantages of the longer life of the wire cloths are to a considerable amount discounted.

The object of the present invention is to make the use of the above mentioned high grade improved steel more economical for the manufacture of machine sieves or wire cloths and the invention consists in making the wires of the warp only of the gauze of a

high grade non-rusting steel which possesses 55 special powers of resistance to wear, while for the weft which is subjected to less strain wires of a lower quality, such for example as the bronze wire which has hitherto been used is employed.

According to the present invention machine sieves are likewise of longer length of life than such in which both the warp and weft are made of high grade improved. They are however as their price is only about 65  $\frac{3}{5}$ ths of that of the latter, considerably cheaper to provide than these and consequently afford very considerable economical advantages.

The improved steels are mainly highly alloyed chromium nickel steels. These are made of different composition according to the special properties which it is desired to obtain and they may also have small quantities of tungsten or vanadium for example 70 75 added to them for the same purpose.

As chromium nickel steels of special properties steels have become for example containing 6-25% Cr, 20-0.5% Ni and up to 1% C, 15-40% Cr, 20-4.0% Ni and up to 1% 80 C, 18-24% Cr, 7-20% Ni, 2-6% Cu and 0.1-0.4% C, 18-30% Cr, 20-4% Ni, 2-4% Mo and 0.1-0.4% C.

They may be used as the material for warp wires for the manufacture of the subject matter of the application. It is obvious of course that the properties of steels so differently alloyed will differ greatly and also the cost of maintenance. Among the chromium nickel steels produced on a manufacturing scale two 85 groups may be selected substantially which possess considerably different chemical and physical properties in addition to differences of structure. The first group of a Martensite or Troostite texture contains 90 steels with a medium amount of chromium and a small amount of nickel. To the second group with an Austenite texture belong steels containing a large amount of chromium and a medium amount of nickel. These 95 are distinguished by great power of resistance to corrosion of every kind and by a very great power of resistance to wear and are particularly suitable as a material for warp wires of the kind herein referred to. The 100 steels of the first group may also be used for the manufacture of warp wires as they can be made rust proof. Although superior to

bronze they do not however possess the same great strength and power of resistance to wear and tear that is possessed by the steels of the second group. On the other hand they 5 are considerably cheaper to manufacture than these. Where high grade nickel steel is used for warp wires, these steels may also be used for the weft.

The present invention may also be used for 10 rotary sieves or wire cloths for other machines than paper making machines as for example for the sieves of machines for the

manufacture of coal dust such as is used for coal dust fire furnaces.

Claim:

Wire gauze for paper making machines comprising warp wires of strong, tough, non-rusting steel and weft wires of lower quality more easily bendable non-rusting material.

In testimony whereof the foregoing specification is signed at Cologne, this 27th day of April, 1926.

ALBERT ELSENHANS.

15

20